

## UNITED STATES PATENT OFFICE

CARL TRENZEN, OF HONNEF-ON-THE-RHINE, GERMANY, ASSIGNOR OF TWO-THIRDS TO  
CARL SCHWARTZ AND G. G. GUTHRIE HUNTER, BOTH OF NEW YORK, N. Y.

## LEPIDOLITE ENAMEL AND METHOD OF PRODUCING SAME

No Drawing. Application filed July 9, 1926, Serial No. 121,502, and in Germany July 10, 1925.

I have discovered that the known material lepidolite is particularly suited for enameling of goods composed of iron and the use of this material has the particular advantage that an undercoat enameling is not necessary. Which, of the mineral components of lepidolite, are responsible for this phenomenon, namely that it is not necessary to burn in an undercoat enamel, has not been possible to ascertain definitely, although it is surmised that the lithium is the cause thereof.

A lepidolite of the following composition:

|                         | Per cent |
|-------------------------|----------|
| Silica                  | 50,38    |
| Alumina                 | 25,96    |
| Iron oxide              | 0,14     |
| Lime                    | 0,08     |
| Magnesium oxide         | 0,03     |
| Lithium oxide           | 4,94     |
| Potash, potassium oxide | 7,21     |
| Sodium oxide            | 5,21     |
| Fluorine                | 7,20     |

is pulverized to the greatest fineness and is, without any other binders, floated with water upon the objects to be enameled and is burned in under a temperature of 1000° C. This forms an enamel firmly adhering to the iron and is completely opaque and very glossy. This coat of enamel is not alone very shock-proof but also, compared with other enamels, extremely resistant to acids.

The enamel burned in at 1000° C. can remain within the furnace without danger for an extended period of time because, when cooling, sufficient opaqueness develops, for which the lithium content is responsible, inasmuch as lithiumoxide is a very marked and suitable crystallizer.

In order to adapt the coefficient of expansion to other coefficients of expansion other substances can be added such as silica, alumina, lime, magnesium oxide on the one side and potash and soda on the other.

The danger of not acquiring a sufficient degree of opaqueness is extremely small on account of the contents of lithiumoxide present.

## Claim:

1. The method of enameling a metal article which consists in applying a coating of pow-

dered lepidolite directly in contact with the metal, and thereafter subjecting the article to a baking temperature.

2. The method of enameling a metal article which consists in applying a coating of powdered lepidolite, carried by a fluent vehicle, directly in contact with the metal, and thereafter subjecting the article to a baking temperature.

3. The method of enameling a metal article which consists in floating directly onto the metal powdered lepidolite, mixed in water, and thereafter subjecting the article to a baking temperature.

4. As an article of manufacture, a piece of metallic stock having baked thereon a coating including lepidolite, said coating having a co-efficient of expansion differing from that of lepidolite and being in direct contact with the stock.

In testimony whereof I affix my signature.  
DR. CARL TRENZEN.

55

60

65

70

75

80

85

90

95

100